

## 1

2,763,921

CORROSION AND IMPACT RESISTANT ARTICLE  
AND METHOD OF MAKING SAME

Percy P. Turner, Jr., and Robert R. Ruppender, Euclid, Ohio, assignors to Thompson Products, Inc., Cleveland, Ohio, a corporation of Ohio

No Drawing. Application January 24, 1952,  
Serial No. 268,146

5 Claims. (Cl. 29—198)

The present invention relates to an impact resistant article, consisting of a refractory metal base and an impact resistant coating.

The instant application is a continuation-in-part of our application, Serial No. 214,116, filed March 6, 1951, entitled "Corrosion and Impact Resistant Article and Method of Making Same."

As explained in the previously identified application, the extensive development in the field of jet engines has necessitated the development of alloys for use in the manufacture of parts for such jet engines which can withstand the extremely high temperatures and oxidizing atmospheres normally present in the operation of turbo-jet engines. Such alloys, to function properly, must have a high strength, toughness, creep-resistance and resistance to the oxidizing gases present in the turbine engine.

One relatively plentiful metal which exhibits good strength, toughness and creep-resistance characteristics is molybdenum. However, the oxidation resistance of molybdenum and alloys containing major amounts of molybdenum is quite poor. Although molybdenum has a melting point in excess of 4500° F., it begins oxidation at temperatures as low as 900° F. The rate of formation of the molybdenum oxide increases with an increase in temperature. Since the molybdenum oxide sublimes, complete disintegration of the molybdenum body will occur in a relatively short time under conditions of high temperature oxidation.

To protect molybdenum bodies against the effects of oxidation, it has been suggested that certain metals or metalloids be coated onto the surface of the molybdenum. Certain coating materials have the ability of forming intermetallic corrosion resistant compounds with the molybdenum surface. In particular, coating materials such as silicon, aluminum, and zirconium form intermetallic compounds with molybdenum. Molybdenum bodies coated with silicon, for example, can withstand thousands of hours of operation above temperatures of red heat without showing any evidence of oxidation of the molybdenum base.

While these intermetallic compound coatings very effectively protect the surface of the molybdenum from oxidation, the intermetallic compounds formed at the surface of the molybdenum are usually quite brittle and liable to failure due to impact. Such impact could result during the operation of gas turbine engines in aircraft due to the presence of foreign objects, even small particles, in the gas streams of the engine. These foreign objects may be received from the outside air, or may result from chipping of the combustion tubes, or from a number of other sources. These particles pass through the turbine at extremely high velocities, on the order of several hundred feet a second. When the foreign objects strike the coated molybdenum part, fracture of the coated surface often results, thereby exposing the refractory metal body to the corrosive atmosphere of the gas stream.

In our aforementioned application, we disclosed that brittle, corrosion resistant surfaces of the type described could be protected against impact by coating the surface with certain nickel-chromium alloys.

## 2

We have now found that substantially improved results can be obtained in practicing the invention described in our aforementioned application by using a plurality of nickel-chromium alloys of differing melting points, but

5 having compositions within the ranges previously described. More particularly, we have found that if the nickel-chromium alloy coating is applied to the surface of the refractory metal article in the form of a matrix of a liquefied nickel-chromium alloy containing dispersed

10 particles of another nickel-chromium alloy having a higher melting point than the matrix, that a superior coating is obtained as compared with the results when a single alloy powder is used. The advantages are particularly marked with respect to the maintenance of a uniform flow of the coating materials at the brazing temperature employed to apply the nickel-chromium alloy to the surface of the refractory body, and the ability to apply thin coatings without the danger of discontinuities.

15 20 An object of the present invention is to provide an improved impact resistant coating to a refractory metal body.

Another object of the present invention is to provide a brazed coating of a nickel-chromium alloy composition in the form of a relatively thin film about a corrosion resistant metal body.

25 Still another object of the present invention is to provide an improved nickel-chromium alloy composition capable of being brazed onto the surface of a refractory metal body in the form of a uniform coating.

30 Still another object of the present invention is to provide an improved method for applying impact resistant coatings to refractory metal bodies.

35 Another object of the present invention is to provide a method for brazing nickel-chromium alloy compositions onto refractory metal articles.

In the method of the present invention, a refractory metal body is provided with an impact resistant coating by applying a coating composition consisting essentially 40 of a liquefied matrix of a nickel-chromium alloy, the matrix containing dispersed particles of a nickel-chromium alloy of higher melting point than the melting point of the matrix.

45 In a preferred embodiment of the present invention, a mechanical mixture of two nickel-chromium alloys having differing melting points, both powders having a particle size on the order of minus 325 mesh, is sprayed onto the surface of the refractory article to be coated. The resulting coated article is then heated to a firing temperature sufficient to just melt the lower melting alloy.

50 Under these conditions, the higher melting particles then begin to dissolve in the liquid phase, the extent of solution being dependent upon the time of treatment. We have found that the best coatings under these conditions 55 are obtained by interrupting the firing cycle before the point of complete solution of the higher melting alloy in the lower melting alloy matrix is reached. While this dissolution is taking place, the semi-fluid coating reacts with the base metal or object being coated, resulting in the formation of a small amount of higher melting alloy at the interface which prevents or hinders the flow of the alloy coating at the given temperature. The resulting coating is then uniform, tight, and integrally bonded to the base metal.

60 65 70 The coatings of the present invention can be applied directly to a refractory metal body such as molybdenum, or alloys of molybdenum containing at least 95% molybdenum. In addition, the alloy coatings of the present invention can also be applied to refractory metal bodies which have been treated, as by reaction with silicon, aluminum, or zirconium, to produce an outer corrosion

resistant layer containing intermetallic compounds of molybdenum and the coating metal.

As another alternative, the molybdenum base may be chromized for the dual purpose of rendering the base metal more oxidation resistant, and to use the chromium as a cushion or buffer layer between the base metal and the brazed coating. Chromium forms a series of solid solutions with molybdenum, but not intermetallic compounds. Furthermore, the brazed coating, when applied to a chromized surface, is more uniform than it is when applied to bare molybdenum since the brazed layer reacts with the chromized layer and tends to eliminate uneven flow during brazing. The chromizing step may be carried out by packing the article to be coated in a layer of granular aluminum oxide which is subsequently surrounded by a pack containing chromium-bearing material such as chromium or ferrochrome. Hydrogen and hydrogen-chloride gas are passed through the pack while maintaining the article at a temperature from 1800° to 2400° F. For the purposes of the present invention the chromizing is continued for a time, usually on the order of two hours, until a chromized coating of from 0.0002 inch to 0.0004 inch is achieved. For the purposes of this invention, the application of chromium by chromizing is definitely superior to the application of chromium by electrodeposition. In chromizing, a substantial thickness of chromium can be built up, and being deposited from a vapor phase reaction, the chromium diffuses into and reacts with the molybdenum base to form a definite bond with the base metal. In addition, chromium deposited from a chromizing process is more reactive than chromium deposited by other processes, and reacts with the subsequently applied brazed coatings.

The nickel-chromium alloys employed in the present invention preferably have analysis within the following ranges:

|    |             |
|----|-------------|
| Mn | 1.0 max.    |
| Si | 0.5 to 5.0  |
| Fe | 1.0 to 5.5  |
| Cr | 8.0 to 20.0 |
| B  | 1.0 to 8.0  |
| Ni | 65 to 90    |
| Zr | 0.05 max.   |
| Ca | 0.20 max.   |
| C  | 0.70 max.   |

The amount of carbon in the alloy is an important consideration, as carbon tends to combine with chromium to form chromium carbide, thereby reducing the effective chromium content. The reduction in effective chromium content reduces the oxidation resistance of the alloy at high temperatures.

The silicon in the above composition may be added as ferro-silicon, and serves to increase the high temperature resistance to oxidation.

Iron imparts fluidity to the alloy and renders it more workable. Iron may be added in the form of ferro-silicon, and this metal is also present in some of the other ingredients as an impurity.

The boron content of the alloy not only lowers the melting point of the alloy but also increases the fluidity of the molten alloy by decreasing its surface tension.

Manganese occurs as an unavoidable impurity and lowers the high temperature resistance of the alloy. The first tenths of one percent are the most detrimental in this respect.

Calcium and zirconium are added to the alloy to act as deoxidizing agents. The more completely deoxidized the alloy, the less susceptible it is to precipitation of oxides at the grain boundaries of the alloy. These two elements serve to increase the high temperature resistance of the alloy.

A preferred coating process consists in mixing two nickel-chromium alloy powders, both having a particle size of minus 325 mesh, and spraying the powdered mix-

ture onto the surface of the article, either in particulated form or in suspension in a binder solution such as a dilute aqueous solution of methyl cellulose. The binder not only helps suspend the alloy particles, but also makes possible the application of tight, thin films of the sprayed mixture which resist cracking and tearing during drying.

The following analyses represent two alloys which have been successfully used in combination to achieve results which are better than the results obtainable when the alloys are used individually.

|    |    | Alloy No. 1 | Alloy No. 2 |
|----|----|-------------|-------------|
| 15 | Mn | 0.01        | 0.01        |
|    | Si | 4.54        | 0.80        |
|    | Fe | 5.02        | 1.05        |
|    | Cr | 14.82       | 18.17       |
|    | B  | 4.53        | 4.86        |
|    | Ni | 70.0        | 74.4        |
| 20 | Zr | 0.01        | 0.01        |
|    | Ca | 0.01        | 0.0         |
|    | C  | 0.68        | 0.24        |

The remainder of the analyses consist of unavoidable impurities.

We prefer to use powdered mixtures containing 40 to 60% of alloy No. 1 with 60 to 40% of alloy No. 2, and specifically about 60% alloy No. 1 and 40% alloy No. 2.

After application of the powdered metal to the surface of the refractory article, the coated article is dried to eliminate free moisture and then heated in a non-oxidizing atmosphere to braze the coating onto the corrosion resistant surface. This brazing operation may be carried out in a dry hydrogen atmosphere, or under vacuum conditions, for a period up to 120 minutes at temperatures from about 1800° to 2300° F.

For the best results, we have found that the brazing temperature should be chosen so that it slightly exceeds the melting point of the lower melting alloy. Some of the discrete particles of the higher melting alloy are dissolved in the liquefied matrix, while others float in the liquid matrix.

The liquid matrix reacts with the refractory metal body to form a high melting alloy at the interface between the refractory metal surface and the coating, thereby preventing or hindering the flow of the alloy coating. The tenacious bond between the brazed coating and the underlying bare molybdenum, chromized molybdenum, or siliconized molybdenum, is due to this reaction between the coating and the base.

In applying these coatings to a molybdenum surface containing an inert oxidation resistant layer, such as a silicide of molybdenum, it is advisable to etch the surface of the article with a reagent such as hydrofluoric acid to make the surface more receptive to the applied coating. A suitable etchant consists of one part hydrofluoric acid (45-55%) with two parts water, the etchant being applied for a period of from 10 to 120 seconds. In the case of silicide coatings, an etching time of about 40 seconds is used while for a chromized coating, an etching time of about 15 seconds is employed.

For best results, the coating should be applied so that the final thickness of the coating is within the range from 0.002 inch to 0.010 inch in thickness, with 0.0030 to 0.0040 inch thickness being an optimum range.

The coatings produced according to the present invention are extremely uniform, smooth and ductile. Surprisingly, the same results are not achieved when using a single alloy having a composition corresponding to the average composition of the mixture of the two alloys.

From the foregoing, it will be appreciated that the novel coatings of the present invention provide increased corrosion and impact resistance to refractory metal articles, making them particularly adaptable to use in high temperature environments and oxidizing conditions, such as occur in turbo-jet engines. The coatings are securely bonded to the underlying refractory metal base, are extremely uniform, smooth and ductile.

It will be understood that modifications and variations may be effected without departing from the scope of the novel concepts of the present invention.

We claim as our invention:

1. An impact and corrosion resistant article comprising a base consisting essentially of molybdenum, and an impact resistant outer surface coating bonded to said base, said coating consisting essentially of a matrix of a nickel-chromium alloy containing dispersed particles of a nickel-chromium alloy having a higher melting point than said matrix, both said matrix and said particles having a composition within the following range:

|    |             |
|----|-------------|
| Mn | 1.0 max.    |
| Si | 0.5 to 5.0  |
| Fe | 1.0 to 5.5  |
| Cr | 8.0 to 20.0 |
| B  | 1.0 to 8.0  |
| Ni | 65 to 90    |
| Zr | 0.05 max.   |
| Ca | 0.20 max.   |
| C  | 0.70 max.   |

2. An impact and corrosion resistant article comprising a base consisting essentially of molybdenum, and an impact resistant outer surface coating bonded to said base, said coating consisting essentially of a matrix of a nickel-chromium alloy containing dispersed particles of a nickel-chromium alloy having a higher melting point than said matrix, both said matrix and said particles having a composition within the following range:

|    |             |
|----|-------------|
| Mn | 1.0 max.    |
| Si | 0.5 to 5.0  |
| Fe | 1.0 to 5.5  |
| Cr | 8.0 to 20.0 |
| B  | 1.0 to 8.0  |
| Ni | 65 to 90    |
| Zr | 0.05 max.   |
| Ca | 0.20 max.   |
| C  | 0.70 max.   |

said coating having a thickness in the range from about 0.002 inch to about 0.010 inch.

3. The method of increasing the corrosion resistance and impact resistance of a molybdenum base which comprises applying over said base a mixture of corrosion resistant nickel-chromium alloys of differing melting points, each of the alloys in said mixture having an analysis in the following range:

|    |             |
|----|-------------|
| Mn | 1.0 max.    |
| Si | 0.5 to 5.0  |
| Fe | 1.0 to 5.5  |
| Cr | 8.0 to 20.0 |
| B  | 1.0 to 8.0  |
| Ni | 65 to 90    |
| Zr | 0.05 max.   |
| Ca | 0.20 max.   |
| C  | 0.70 max.   |

each of said alloys constituting substantial percentages of the total mixture, heating the resulting composite article to a temperature and for a time sufficient to render the lower melting alloy in said mixture molten, said temperature being insufficiently high to melt the higher melting alloy of said mixture, maintaining said lower melting alloy molten until said alloy reacts with the underlying surface and dissolves some of said higher melting alloy, terminating said heating before all of said higher melting alloy is dissolved and cooling the composite article to provide a uniform, smooth coating over said molybdenum base consisting of a matrix of said lower melting alloy having dispersed therein undissolved particles of said higher melting alloy.

4. The method of increasing the corrosion resistance and impact resistance of a molybdenum base which comprises applying over said base a mixture of corrosion re-

sistant nickel-chromium alloys, each of the alloys in said mixture having an analysis in the following range:

|    |             |
|----|-------------|
| Mn | 1.0 max.    |
| Si | 0.5 to 5.0  |
| Fe | 1.0 to 5.5  |
| Cr | 8.0 to 20.0 |
| B  | 1.0 to 8.0  |
| Ni | 65 to 90    |
| Zr | 0.05 max.   |
| Ca | 0.20 max.   |
| C  | 0.70 max.   |

said mixture containing from 60 to 40% by weight of a higher melting alloy and from 40 to 60% by weight of a lower melting alloy, heating the resulting composite article to a temperature and for a time sufficient to render the lower melting alloy in said mixture molten, said temperature being insufficiently high to melt the higher melting alloy of said mixture, maintaining said lower melting alloy molten until said alloy reacts with the underlying surface and dissolves some of said higher melting alloy, terminating said heating before all of said higher melting alloy is dissolved and cooling the composite article to provide a uniform, smooth coating over said molybdenum base consisting of a matrix of said lower melting alloy having dispersed therein undissolved particles of said higher melting alloy.

5. The method of increasing the corrosion resistance and impact resistance of a molybdenum base which comprises chromizing said molybdenum base, applying over the resulting chromized surface a mixture of corrosion-resistant nickel-chromium alloys of differing melting points, each of the alloys in said mixture having an analysis in the following range:

|    |             |
|----|-------------|
| Mn | 1.0 max.    |
| Si | 0.5 to 5.0  |
| Fe | 1.0 to 5.5  |
| Cr | 8.0 to 20.0 |
| B  | 1.0 to 8.0  |
| Ni | 65 to 90    |
| Zr | 0.05 max.   |
| Ca | 0.20 max.   |
| C  | 0.70 max.   |

each of said alloys constituting substantial percentages of the total mixture, heating the resulting composite article to a temperature and for a time sufficient to render the lower melting alloy in said mixture molten, said temperature being insufficiently high to melt the higher melting alloy of said mixture, maintaining said lower melting alloy molten until said alloy reacts with the underlying surface and dissolves some of said higher melting alloy, terminating said heating before all of said higher melting alloy is dissolved and cooling the composite article to provide a uniform, smooth coating over said molybdenum base consisting of a matrix of said lower melting alloy having dispersed therein undissolved particles of said higher melting alloy.

#### References Cited in the file of this patent

#### UNITED STATES PATENTS

|           |                |               |
|-----------|----------------|---------------|
| 1,365,499 | Kelley         | Jan. 11, 1921 |
| 1,650,979 | Brace          | Nov. 29, 1927 |
| 2,162,253 | Grossman       | June 13, 1939 |
| 2,190,840 | Kay            | Feb. 20, 1940 |
| 2,323,169 | Wagenhals      | June 29, 1943 |
| 2,375,154 | Volterra       | May 1, 1945   |
| 2,401,040 | Becker         | May 28, 1946  |
| 2,455,804 | Ransley et al. | Dec. 7, 1948  |
| 2,520,373 | Price          | Aug. 29, 1950 |
| 2,587,275 | Bash           | Feb. 26, 1952 |
| 2,697,130 | Korbelak       | Dec. 14, 1954 |

#### FOREIGN PATENTS

|         |               |               |
|---------|---------------|---------------|
| 474,064 | Great Britain | Jan. 17, 1936 |
| 487,263 | Great Britain | June 17, 1938 |